

Oct. 21, 1941.

S. G. ROSS

2,259,586

METHOD OF TREATING UNATTACHED SOLES

Filed Nov. 15, 1939

Fig1



Fig2



Fig3



INVENTOR  
Simon G. Ross  
By his Attorney  
Victor Cobb

## UNITED STATES PATENT OFFICE

2,259,586

## METHOD OF TREATING UNATTACHED SOLES

Simon G. Ross, Lynn, Mass., assignor to United Shoe Machinery Corporation, Borough of Flemington, N. J., a corporation of New Jersey

Application November 15, 1939, Serial No. 304,577

3 Claims. (Cl. 12—146)

This invention relates to methods of treating leather articles and is concerned chiefly with the problems of tempering unattached soles with liquid. The invention is hereinafter set forth, by way of example, with reference to treating outsoles but it is not limited to outsole treatment since in some circumstances it may be applicable to the treatment of other articles made of leather.

The invention is predicated upon the fact that when leather is in a condition that is considered dry from the standpoint of shoemaking, its pores contain air in addition to residual quantities of tanning substances. Consequently, to enable a liquid such as water to bring a sole into a satisfactory state of temper for various shoemaking operations, including channeling, rounding, laying, stitching, or attaching with cement, channel-closing and leveling, it is necessary to remove a considerable proportion of the air initially in the leather, much of which is trapped in the pores by the residual tanning substances. It is only with difficulty that air may be removed through the grain side of leather, since that side is much more dense than the flesh side. Again, if a marginal band of the flesh side has been fleshed and coated with attaching cement the latter forms a barrier by which air is trapped in the pores covered thereby. These conditions of inequality of perviousness have heretofore rendered tempering difficult and unsatisfactory in that some parts of a sole may become sodden with too much moisture before other parts have absorbed enough moisture to render them pliant.

To shorten the time required to temper a sole and at the same time to facilitate the dispersion of a tempering liquid through the soles, the invention provides an improved method which consists in puncturing the flesh side of a sole at many points without puncturing the grain side thereof, immersing the sole in a tempering liquid, and removing the sole from the liquid before any part of it becomes sodden. The puncturing may be done either by pricking many small holes in the flesh side with needle-points or by scoring the flesh side with many fine cuts as with a knife-edge or a group of them. If the punctures are formed by scoring, the scoring cuts need not all be parallel and need not all extend in one general direction but may intersect one another, the essential consideration being that they shall break into the pores in the flesh side of the leather and loosen the residual tanning substances to a degree that will release much of the air that would otherwise remain trapped in the leather to repell tempering liquid seeking

to enter the pores. The pricking procedure has the same releasing effect, and both have a flexing effect that is not lost when the tempering moisture has evaporated from the sole.

If a sole is to be attached with cement alone, a strong attaching bond requires the cement to be applied thereto while the sole is dry. Moreover, the procedure requires shaping the sole to final configuration, fleshing it and roughing a marginal band thereof before applying attaching cement to the latter. According to the novel method disclosed herein, the puncturing or scoring of the flesh side of the sole will be done after the attaching cement has been applied and has grown hard, and some of the punctures or scoring cuts will break through the band of cement. Consequently, when the sole is thereafter subjected to a tempering fluid, the latter will pass through the band of cement and some of the air in the pores of the cement-coated margin of leather may escape through the breaks in the cement.

Again, some manufacturers temper soles in liquid at atmospheric pressure, while others, to shorten the time required for tempering, speed the efflux of air from the pores by subjecting the tempering liquid to minus pressure while the sole or soles are immersed therein and this stage of minus pressure may be followed by a stage of atmospheric pressure with or without a subsequent stage of plus pressure or another stage of minus pressure. For the purposes of this description, minus pressure is to be understood as any pressure below atmospheric pressure and plus pressure is to be understood as any pressure above atmospheric pressure, regardless of whether this classification is the one commonly recognized by scientific authorities.

If attaching cement be applied to a sole when the latter is not in temper to avoid impairing the efficiency of the cement, and if approximately uniform tempering of coated and uncoated portions of a sole is desired, it may be obtained by utilizing the principles of the present invention according to the following method of procedure which consists in coating only a marginal band of the flesh side of a sole with attaching cement, permitting the cement to dry or harden thereon, puncturing the band of cement at many points either by pricking many small holes through it or by scoring it with many fine lines with much or little penetration of the flesh part of the band, immersing the sole in a tempering liquid, and removing the sole from the liquid before the uncoated area of the flesh side becomes sodden.

Here also, the tempering liquid may remain at atmospheric pressure or may be subjected to minus pressure with or without being subjected to plus pressure during the period of immersion, but regardless of pressure changes, the puncturing of the barrier of cement will facilitate the efflux of air therethrough and the influx of liquid to replace the air in the pores under the band of cement. Consequently, even though the barrier of cement may not cover the middle area of the sole, the preliminary puncturing of the band of cement, according to this procedure will, in a great measure, counteract the initial difference between the coated area and the uncoated area with respect to their ability to emit air from the pores and admit a tempering fluid into them. Approximation of uniformity in this respect will be further promoted by subjecting the tempering fluid to a stage of minus pressure by which the air in the pores of the coated band will be withdrawn quickly through the punctures in the barrier of cement, while the air in the uncoated area is being withdrawn through the unpunctured surface thereof.

The procedure last described is predicated upon a preference for approximately uniform tempering of coated and uncoated areas of a sole, but to satisfy a demand for more temper of a selected area than all other areas the selected area may be punctured accordingly and the other areas provided with fewer punctures or none at all, as circumstances may require.

The invention provides still another improved procedure which consists in coating with attaching cement a marginal band of the flesh side of a fleshed and roughed sole, permitting the cement to dry or harden thereon, puncturing both the coated area and the uncoated area of the forepart and the shank, but preferably not the heel-seat (because not much moisture is ever desired in the heel-seat), immersing the sole in a tempering liquid, and removing the sole from the tempering liquid before it becomes sodden. Even though this latter procedure may result in greater intake of liquid in the uncoated portions of the forepart and the shank than in the cement-coated portions thereof, capillary action will transfer some of the absorbed liquid from the uncoated area to the coated area and thus, in some measure, increases the tempered condition of the coated area before the subsequent shoemaking operations that require the sole to be in temper have been performed.

To practice any or all of the improvements herein set forth does not require any special apparatus unless the work is to be subjected to changes of fluid pressure during the tempering operation. One type of apparatus designed to speed the tempering of soles by subjecting the tempering liquid to minus pressure with or without a stage of plus pressure is illustrated in Figs. 3 and 4 of United States Letters Patent No. 1,948,994, granted February 27, 1934, on application of H. S. Pochin. The pressures of the tempering liquid may be regulated at will in such apparatus.

The puncturing of the flesh side of the leather or of the coating of cement, or both, may be much or little, deep or shallow, according to the character of the leather, the character of the cement or according to the results desired. Accordingly, to obtain uneven tempering and to control localization thereof in selected portions of a sole, the invention provides still another improved procedure which consists in punctur-

ing the flesh side of a sole at many points in a certain selected area where the greatest degree of tempering is desired, puncturing one or more other areas at fewer points per unit of area, 5 omitting all puncturing in an area where the least moisture is desired, immersing the sole thus unevenly or unequally punctured in a tempering liquid, and removing the sole from the liquid before it becomes sodden in the most punctured 10 area. Such a procedure will produce tempering of different degrees according to whether the area affected has been punctured or not, and if punctured at all, according to whether the puncturing is much or little.

15 Referring to the drawing:

Fig. 1 represents the flesh side of a block sole, a limited area of which has been punctured with many small holes to speed impregnation with the tempering fluid;

Fig. 2 represents the flesh side of a sole that has been fleshed and shaped to final configuration, a marginal band thereof being roughed and coated with attaching cement and a limited area thereof being punctured with many small holes some of which extend through the band of cement;

Fig. 3 represents a sole likewise shaped to final configuration, a marginal band thereof being roughed and coated with attaching cement and punctured with many small holes.

In the manufacture of welt shoes, it is customary to use an outsole 10 of the block type (Fig. 1) to be shaped after it is attached with stitches. Soles of this type are commonly tempered with water before being laid. The degree of temper should be enough to facilitate rough rounding, channeling and all making operations to be performed before the usual bottom-finishing operations. Not much tempering is required at the toe end, or at the heel end, but the shank and region of the ball should be well tempered to facilitate conforming the sole to the corresponding regions of a shoe in the sole-laying stage and again in the leveling stage. Accordingly, to 40 insure a greater degree of temper in the ball and shank areas, the present invention provides for a greater degree of impregnation with a tempering fluid in consequence of puncturing the flesh side of these areas with many small holes indicated by dots 11. This puncturing may be done with one or more strokes of a block (not shown) provided with many small sharp points that will penetrate the sole from the flesh side without going through the sole to the grain side. 45 After the sole is so punctured, it will be subjected to a tempering operation which may consist merely in immersing the sole in water or other tempering liquid at atmospheric pressure for a suitable length of time preferably not enough to render the sole sodden. The intake of the tempering liquid in the punctured area will be greater than that in the unpunctured areas and the degrees of temper in the punctured and unpunctured areas will differ accordingly.

On the other hand, if more rapid tempering is desired, the sole may be subjected to one or more stages of minus pressure with or without one or more stages of positive pressure, or one or more stages of atmospheric pressure, while immersed in a bath of tempering liquid in an apparatus utilizing the principles disclosed in the above-mentioned Letters Patent 1,948,994. When those principles are utilized air is withdrawn from the pores of the leather by the minus pressure and the tempering liquid readily enters the leather

through the punctures and is dispersed laterally from them.

If a sole such as that indicated at 12 in Fig. 2 is to be attached with cement alone, it will first be fleshed, then shaped to final configuration as represented in this figure, and a marginal band of its attaching face will be roughed and thereafter coated with attaching cement insoluble in water. The cement is indicated by shading 13. When this band of cement has grown hard, any selected area of the sole where flexibility is particularly desired may be punctured with many small holes, again indicated by dots 11. In this example some of the punctures are localized in the cemented band, and of these some are more closely spaced than others to insure a greater degree of temper in the shank than in the forepart. Other punctures more widely spaced are localized in the uncoated area of the ball region of the forepart. The punctures in the band of cement not only permit an influx of the tempering fluid but also permit emission of air that would otherwise be trapped in the pores of the band so coated. When a sole thus prepared is subsequently subjected to a tempering fluid, it will derive various degrees of temper in different areas according to the location of the cement, the location of the punctures and the spacing of the punctures, one from another.

If desired, the punctures may be restricted to the cement-coated band as represented in Fig. 3, in which the sole 14 is first fleshed, then shaped to final configuration, and a marginal band of its attaching face roughed and thereafter coated with attaching cement 13 as described with reference to Fig. 2. After this band of the cement has grown hard, it may be punctured with enough small holes, indicated by dots 15, to admit quantities of tempering fluid that will not dissolve the cement but will temper the margins to about the same degree as the uncoated area. Since no sole requires much, if any flexibility or

temper at its extremities, the punctures may be omitted accordingly, and such omission is represented in all the figures. Once the punctures have been located according to the results desired, the sole will be impregnated with a tempering fluid having the characteristics above specified.

Having thus described my invention, what I claim as new and desire to secure by Letters 10 Patent of the United States is:

1. That improvement in methods of treating articles of sole-leather which consists in coating an area of the flesh side of an article with an adhesive substance, permitting the adhesive 15 coating to dry or harden thereon, puncturing the coating of said substance at many points to enable air and liquid to flow readily through it, immersing the article in a bath of tempering liquid in which said adhesive substance is insoluble, and removing it from the bath before it becomes sodden.

2. That improvement in methods of treating unattached leather soles which consists in coating only a marginal band of the flesh side of a sole with attaching cement insoluble in water, permitting the coating of cement to dry or harden thereon, puncturing the band of cement and the leather thereunder at many points to facilitate the efflux of air from the pores in said 25 band and the influx of liquid into said pores, immersing the sole in a bath of water, and removing the sole from said bath before it becomes sodden.

3. The improved method set forth in claim 2 30 supplemented by the intermediate step of subjecting the water to minus pressure while the sole is immersed therein to withdraw air from the pores in said band and through the openings punctured in the cement with which said 35 band is coated.

SIMON G. ROSS.